



US008574804B2

(12) **United States Patent**  
**Chen et al.**

(10) **Patent No.:** **US 8,574,804 B2**  
(b5) **Date of Patent:** **Nov. 5, 2013**

(54) **TONER COMPOSITIONS AND PROCESSES**

(75) Inventors: **Allan K. Chen**, Oakville (CA); **Santiago Faucher**, Oakville (CA); **Edward Graham Zwart**, Mississauga (CA); **Kimberly D. Nosella**, Mississauga (CA); **Daryl W. Vanbesien**, Burlington (CA)

(73) Assignee: **Xerox Corporation**, Norwalk, CT (US)

(\*) Notice: Subject to any disclaimer, the term of this patent is extended or adjusted under 35 U.S.C. 154(b) by 553 days.

(21) Appl. No.: **12/869,022**

(22) Filed: **Aug. 26, 2010**

(65) **Prior Publication Data**

US 2012/0052433 A1 Mar. 1, 2012

(51) **Int. Cl.**

**G03G 9/00** (2006.01)

(52) **U.S. Cl.**

USPC ..... **430/110.2**; 430/108.4; 430/109.1

(58) **Field of Classification Search**

USPC ..... **430/108.4**, 110.2, 109.1

See application file for complete search history.

(56) **References Cited**

## U.S. PATENT DOCUMENTS

|             |         |                  |
|-------------|---------|------------------|
| 3,590,000 A | 6/1971  | Palermiti et al. |
| 3,655,374 A | 4/1972  | Palermiti et al. |
| 3,720,617 A | 3/1973  | Chatterji et al. |
| 3,847,604 A | 11/1974 | Hagenbach et al. |
| 3,944,493 A | 3/1976  | Jadwin et al.    |
| 3,983,045 A | 9/1976  | Jugle et al.     |
| 4,007,293 A | 2/1977  | Mincer et al.    |
| 4,079,014 A | 3/1978  | Burness et al.   |
| 4,295,990 A | 10/1981 | Verbeek et al.   |

|             |         |                            |
|-------------|---------|----------------------------|
| 4,394,430 A | 7/1983  | Jadwin et al.              |
| 4,560,635 A | 12/1985 | Hoffend et al.             |
| 4,935,326 A | 6/1990  | Creatura et al.            |
| 4,937,166 A | 6/1990  | Creatura et al.            |
| 5,236,629 A | 8/1993  | Mahabadi et al.            |
| 5,278,020 A | 1/1994  | Grushkin et al.            |
| 5,290,654 A | 3/1994  | Sacripante et al.          |
| 5,302,486 A | 4/1994  | Patel et al.               |
| 5,308,734 A | 5/1994  | Sacripante et al.          |
| 5,330,874 A | 7/1994  | Mahabadi et al.            |
| 5,344,738 A | 9/1994  | Kmiecik-Lawrynowicz et al. |
| 5,346,797 A | 9/1994  | Kmiecik-Lawrynowicz et al. |
| 5,348,832 A | 9/1994  | Sacripante et al.          |
| 5,364,729 A | 11/1994 | Kmiecik-Lawrynowicz et al. |
| 5,366,841 A | 11/1994 | Patel et al.               |
| 5,370,963 A | 12/1994 | Patel et al.               |
| 5,403,693 A | 4/1995  | Patel et al.               |
| 5,405,728 A | 4/1995  | Hopper et al.              |
| 5,418,108 A | 5/1995  | Kmiecik-Lawrynowicz et al. |
| 5,496,676 A | 3/1996  | Croucher et al.            |
| 5,501,935 A | 3/1996  | Patel et al.               |
| 5,527,658 A | 6/1996  | Hopper et al.              |
| 5,585,215 A | 12/1996 | Ong et al.                 |
| 5,650,255 A | 7/1997  | Ng et al.                  |
| 5,650,256 A | 7/1997  | Veregin et al.             |
| 5,723,253 A | 3/1998  | Higashino et al.           |
| 5,744,520 A | 4/1998  | Kmiecik-Lawrynowicz et al. |
| 5,747,215 A | 5/1998  | Ong et al.                 |
| 5,763,133 A | 6/1998  | Ong et al.                 |
| 5,766,818 A | 6/1998  | Smith et al.               |
| 5,804,349 A | 9/1998  | Ong et al.                 |
| 5,827,633 A | 10/1998 | Ong et al.                 |

(Continued)

*Primary Examiner* — Thorl Chea(74) *Attorney, Agent, or Firm* — MDIP LLC(57) **ABSTRACT**

Toners are provided, which possess low melt properties capable of producing a low gloss finish. The toners include a core and a shell. The shell includes a crystalline resin. The core may include at least one amorphous resin, an optional crystalline resin, an optional wax, and an optional colorant.

**20 Claims, 2 Drawing Sheets**

---

| (56)                  | <b>References Cited</b> |                      |                  |                                    |
|-----------------------|-------------------------|----------------------|------------------|------------------------------------|
| U.S. PATENT DOCUMENTS |                         |                      |                  |                                    |
| 5,840,462 A           | 11/1998                 | Foucher et al.       | 6,730,450 B1     | 5/2004 Moffat et al.               |
| 5,853,943 A           | 12/1998                 | Cheng et al.         | 6,743,559 B2     | 6/2004 Combes et al.               |
| 5,853,944 A           | 12/1998                 | Foucher et al.       | 6,756,176 B2     | 6/2004 Stegamat et al.             |
| 5,863,698 A           | 1/1999                  | Patel et al.         | 6,780,500 B2     | 8/2004 Dumouchel                   |
| 5,869,215 A           | 2/1999                  | Ong et al.           | 6,830,860 B2     | 12/2004 Sacripante et al.          |
| 5,902,710 A           | 5/1999                  | Ong et al.           | 7,029,817 B2     | 4/2006 Robinson et al.             |
| 5,910,387 A           | 6/1999                  | Mychajlowskij et al. | 7,247,413 B2     | 7/2007 Kido et al.                 |
| 5,916,725 A           | 6/1999                  | Patel et al.         | 7,329,476 B2     | 2/2008 Sacripante et al.           |
| 5,919,595 A           | 7/1999                  | Mychajlowskij et al. | 2006/0216626 A1  | 9/2006 Sacripante et al.           |
| 5,925,488 A           | 7/1999                  | Patel et al.         | 2006/0222991 A1  | 10/2006 Sacripante et al.          |
| 5,977,210 A           | 11/1999                 | Patel et al.         | 2008/0107989 A1  | 5/2008 Sacripante et al.           |
| 5,994,020 A           | 11/1999                 | Patel et al.         | 2008/0107990 A1  | 5/2008 Field et al.                |
| 6,004,714 A           | 12/1999                 | Ciccarelli et al.    | 2008/0153027 A1  | 6/2008 Veregin et al.              |
| 6,190,815 B1          | 2/2001                  | Ciccarelli et al.    | 2008/0236446 A1  | 10/2008 Zhou et al.                |
| 6,593,049 B1          | 7/2003                  | Veregin et al.       | 2009/0047593 A1  | 2/2009 Vanbesien et al.            |
|                       |                         |                      | 2009/0208864 A1  | 8/2009 Zhou et al.                 |
|                       |                         |                      | 2009/0246680 A1  | 10/2009 Chung et al.               |
|                       |                         |                      | 2010/0330486 A1* | 12/2010 Zhou et al. .... 430/108.4 |

\* cited by examiner

**F/G. 1**



FIG. 2

## 1

## TONER COMPOSITIONS AND PROCESSES

## BACKGROUND

This disclosure is generally directed to toner processes, and more specifically, emulsion aggregation and coalescence processes, as well as toner compositions formed by such processes and development processes using such toners for use with electrophotographic copying or printing apparatus.

Emulsion aggregation/coalescing processes for the preparation of toners are illustrated in a number of patents, such as U.S. Pat. Nos. 5,290,654, 5,278,020, 5,308,734, 5,370,963, 5,344,738, 5,403,693, 5,418,108, 5,364,729, and 5,346,797; and also of interest may be U.S. Pat. Nos. 5,348,832; 5,405,728; 5,366,841; 5,496,676; 5,527,658; 5,585,215; 5,650,255; 5,650,256; 5,501,935; 5,723,253; 5,744,520; 5,763,133; 5,766,818; 5,747,215; 5,827,633; 5,853,944; 5,804,349; 5,840,462; 5,869,215; 5,863,698; 5,902,710; 5,910,387; 5,916,725; 5,919,595; 5,925,488 and 5,977,210. Other patents disclosing exemplary emulsion aggregation/coalescing processes include, for example, U.S. Pat. Nos. 6,730,450, 6,743,559, 6,756,176, 6,780,500, 6,830,860, and 7,029,817. The disclosures of each of the foregoing patents and publications are hereby incorporated by reference in their entirety.

Some emulsion aggregation (EA) toners are based on a mixture of amorphous and crystalline polyesters. Such toners may also have a core-shell configuration. Where both a core and shell are present, the core may include both amorphous and crystalline polyesters, with the shell having only an amorphous polyester. For many EA toners, there is a trade-off between obtaining desirable gloss and Minimum Fix (or Fusing) Temperature (MFT) characteristics. For example, many EA toners have high gloss and low melt properties. However, for applications where a lower gloss is desired, difficulties may arise in forming a toner having a lower gloss which still exhibits ultra low melt properties.

Improved toners and methods for their production thus remain desirable.

## SUMMARY

The present disclosure provides toners and processes for making same. In embodiments, a toner of the present disclosure may include particles including a core including at least one amorphous polyester resin, an optional crystalline resin, a colorant, and an optional wax; and a shell including at least one amorphous resin in combination with at least one crystalline resin, the at least one crystalline resin being present in an amount of from about 1% to about 50% by weight of the shell, wherein the toner has a gloss of from about 25 ggu to about 85 ggu.

In other embodiments, a toner of the present disclosure may include particles including a core including at least one amorphous polyester resin, an optional crystalline polyester resin, at least one wax, and a colorant; and a shell including at least one amorphous resin in combination with at least one crystalline resin, the at least one crystalline resin being present in an amount of from about 1% to about 50% by weight of the shell, wherein the toner has a gloss of from about 35 ggu to about 75 ggu.

In other embodiments, a toner of the present disclosure may include a core including at least one amorphous polyester resin, from about 1% to about 24% by weight of at least one wax, and at least one colorant; and a shell including from about 50% to about 90% by weight of at least one amorphous

## 2

polyester resin, and from about 10% to about 50% of at least one crystalline resin, wherein the toner has a gloss from about 25 ggu to about 85 ggu.

## BRIEF DESCRIPTION OF THE FIGURES

Various embodiments of the present disclosure will be described herein below with reference to the figure wherein:

FIG. 1 is a graph depicting the gloss of a toner of the present disclosure at various fusing roll temperatures as compared to toners of the prior art; and

FIG. 2 is a graph depicting crease area of a toner of the present disclosure at various fusing roll temperatures as compared to toners of the prior art.

## DETAILED DESCRIPTION

In accordance with the present disclosure, low melt EA toners are provided which include an amorphous resin, a crystalline resin, optionally a pigment, and optionally a wax. The toners of the present disclosure possess good fixing properties. The toners of the present disclosure also exhibit tunable gloss properties, including low gloss and matte finishes, while maintaining low melt properties. Thus, toners of the present disclosure may be utilized to form ultra low melt toners having high gloss, as well as those that are low gloss, i.e., produce matte finishes. In embodiments, the toners of the present disclosure possess a core-shell configuration, with the shell including at least one amorphous resin and a crystalline resin.

## Resin

Toners of the present disclosure may include any latex resin suitable for use in forming a toner. Such resins, in turn, may be made of any suitable monomer. Suitable monomers useful in forming the resin include, but are not limited to, acrylonitriles, diols, diacids, diamines, diesters, diisocyanates, combinations thereof, and the like. Any monomer employed may be selected depending upon the particular polymer to be utilized.

Any toner resin may be utilized in the processes of the present disclosure. Such resins, in turn, may be made of any suitable monomer or monomers via any suitable polymerization method. In embodiments, the resin may be prepared by a method other than emulsion polymerization. In further embodiments, the resin may be prepared by condensation polymerization.

In embodiments, the polymer utilized to form the resin may be a polyester resin. Suitable polyester resins include, for example, sulfonated, non-sulfonated, crystalline, amorphous, combinations thereof, and the like. The polyester resins may be linear, branched, combinations thereof, and the like. Polyester resins may include, in embodiments, those resins described in U.S. Pat. Nos. 6,593,049 and 6,756,176, the disclosures of each of which are hereby incorporated by reference in their entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, a resin utilized in forming a toner may include an amorphous polyester resin. In embodiments, the resin may be a polyester resin formed by reacting a diol with a diacid or diester in the presence of an optional catalyst.

Examples of organic diols selected for the preparation of amorphous resins include aliphatic diols with from about 2 to about 36 carbon atoms, such as 1,2-ethanediol, 1,3-propanediol, 1,4-butanediol, 1,5-pentanediol, 1,6-hexanediol,

3

1,7-heptanediol, 1,8-octanediol, 1,9-nanediol, 1,10-decanediol, 1,12-dodecanediol, and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol is, for example, selected in an amount of from about 45 to about 50 mole percent of the resin, and the alkali sulfo-aliphatic diol can be selected in an amount of from about 1 to about 10 mole percent of the resin.

Examples of diacid or diesters selected for the preparation of the amorphous polyester include dicarboxylic acids or

4

copoly(propoxylated bisphenol A co-terephthalate), a terpoly (propoxylated bisphenol A co-fumarate)-terpoly(propoxylated bisphenol A co-terephthalate)-terpoly-(propoxylated bisphenol A co-dodecylsuccinate), and combinations thereof.

In embodiments, the amorphous resin utilized in the core may be linear.

In embodiments, a suitable amorphous resin may include alkoxylated bisphenol A fumarate/terephthalate based polyesters and copolyester resins. In embodiments, a suitable amorphous polyester resin may be a copoly(propoxylated bisphenol A co-fumarate)-copolyp(propoxylated bisphenol A co-terephthalate) resin having the following formula (I):



diesters selected from the group consisting of terephthalic acid, phthalic acid, isophthalic acid, fumaric acid, maleic acid, itaconic acid, succinic acid, succinic anhydride, dodecylsuccinic acid, dodecylsuccinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, dimethyl dodecylsuccinate, and mixtures thereof. The organic diacid or diester is selected, for example, from about 45 to about 52 mole percent of the resin.

Examples of suitable polycondensation catalyst for either the amorphous polyester resin include tetraalkyl titanates, dialkyltin oxide such as dibutyltin oxide, tetraalkyltin such as dibutyltin dilaurate, dialkyltin oxide hydroxide such as butyltin oxide hydroxide, aluminum alkoxides, alkyl zinc, dialkyl zinc, zinc oxide, stannous oxide, or mixtures thereof; and which catalysts are selected in amounts of, for example, from about 0.01 mole percent to about 5 mole percent based on the starting diacid or diester used to generate the polyester resin.

In embodiments, suitable amorphous resins include polyesters, polyamides, polyimides, polyolefins, polyethylene, polybutylene, polyisobutyrate, ethylene-propylene copolymers, ethylene-vinyl acetate copolymers, polypropylene, combinations thereof, and the like. Examples of amorphous resins which may be utilized include amorphous polyester resins. Exemplary amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), a copoly(propoxylated bisphenol A co-fumarate)-

25 wherein R may be hydrogen or a methyl group, and m and n represent random units of the copolymer and m may be from about 2 to 10, and n may be from about 2 to 10.

about 2 to 10, and it may be from about 2 to 10.

An example of a linear copoly(propoxylated bisphenol A co-fumarate)-copoly(propoxylated bisphenol A co-terephthalate) which may be utilized as a latex resin is available under the trade name SPARII from Resana S/A Industrias Quimicas, Sao Paulo Brazil. Other propoxylated bisphenol A fumarate resins that may be utilized and are commercially available include GTUF and FPESL-2 from Kao Corporation, Japan, and EM181635 from Reichhold, Research Triangle Park, N.C. and the like.

A-terephthalate), poly(propoxylated bisphenol A-isophthalate), poly(propoxylated bisphenol A-dodecenylsuccinate), SPAR (Dixie Chemicals), BECKOSOL (Reichhold Inc), ARAKOTE (Ciba-Geigy Corporation), HETRON (Ashland Chemical), PARAPLEX (Rohm & Haas), POLYLITE (Reichhold Inc), PLASTHALL (Rohm & Haas), CYGAL (American Cyanamide), ARMCO (Armco Composites), ARPOL (Ashland Chemical), CELANEX (Celanese Eng), RYNITE (DuPont), STYPOL (Freeman Chemical Corporation) and combinations thereof. The resins can also be functionalized, such as carboxylated, sulfonated, or the like, and particularly such as sodio sulfonated, if desired.

The amorphous polyester resin may be a branched resin. As used herein, the terms "branched" or "branching" includes branched resin and/or cross-linked resins. Branching agents for use in forming these branched resins include, for example, a multivalent polyacid such as 1,2,4-benzene-tricarboxylic acid, 1,2,4-cyclohexanetricarboxylic acid, 2,5,7-naphthalenetricarboxylic acid, 1,2,4-naphthalenetricarboxylic acid, 1,2,5-hexanetricarboxylic acid, 1,3-dicarboxyl-2-methyl-2-methylene-carboxylpropane, tetra(methylene-carboxyl) methane, and 1,2,7,8-octanetetracarboxylic acid, acid anhydrides thereof, and lower alkyl esters thereof; 1 to about 6 carbon atoms; a multivalent polyol such as sorbitol, 1,2,3,6-hexanetetrol, 1,4-sorbitane, pentaerythritol, dipentaerythritol, tripentaerythritol, sucrose, 1,2,4-butanetriol, 1,2,5-pentatriol, glycerol, 2-methylpropanetriol, 2-methyl-1,2,4-butanetriol, trimethylethane, trimethylolpropane, 1,3,5-trihydroxymethylbenzene, mixtures thereof, and the like. The branching agent amount selected is, for example, from about 0.1 to about 5 mole percent of the resin.

Linear or branched unsaturated polyesters selected for reactions include both saturated and unsaturated diacids (or anhydrides) and dihydric alcohols (glycols or diols). The resulting unsaturated polyesters are reactive (for example, crosslinkable) on two fronts: (i) unsaturation sites (double bonds) along the polyester chain, and (ii) functional groups such as carboxyl, hydroxy, and the like groups amenable to acid-base reactions. Typical unsaturated polyester resins may be prepared by melt polycondensation or other polymerization processes using diacids and/or anhydrides and diols.

In embodiments, a suitable amorphous resin utilized in a toner of the present disclosure may be a low molecular weight amorphous resin, sometimes referred to, in embodiments, as an oligomer, having a weight average molecular weight ( $M_w$ ) of from about 500 daltons to about 10,000 daltons, in embodiments from about 1000 daltons to about 5000 daltons, in other embodiments from about 1500 daltons to about 4000 daltons.

The low molecular weight amorphous resin may possess a glass transition temperature of from about 58.5° C. to about 66° C., in embodiments from about 60° C. to about 62° C.

The low molecular weight amorphous resin may possess a softening point of from about 105° C. to about 118° C., in embodiments from about 107° C. to about 109° C.

In further embodiments, the combined amorphous resins may have a melt viscosity of from about 10 to about 1,000,000 Pa\*S at about 130° C., in embodiments from about 50 to about 100,000 Pa\*S.

The monomers used in making the selected amorphous polyester resin are not limited, and the monomers utilized may include any one or more of, for example, ethylene, propylene, and the like. Known chain transfer agents, for example dodecanethiol or carbon tetrabromide, can be utilized to control the molecular weight properties of the polyester. Any suitable method for forming the amorphous or crystalline polyester from the monomers may be used without restriction.

In other embodiments, an amorphous resin utilized in forming a toner of the present disclosure may be a high molecular weight amorphous resin. As used herein, the high molecular weight amorphous polyester resin may have, for example, a number average molecular weight ( $M_n$ ), as measured by gel permeation chromatography (GPC) of, for example, from about 1,000 to about 10,000, in embodiments from about 2,000 to about 9,000, in embodiments from about 3,000 to about 8,000, and in embodiments from about 6,000 to about 7,000. The weight average molecular weight ( $M_w$ ) of the resin is greater than 45,000, for example, from about 45,000 to about 150,000, in embodiments from about 50,000 to about 100,000, in embodiments from about 63,000 to about 94,000, and in embodiments from about 68,000 to about 85,000, as determined by GPC using polystyrene standard. The polydispersity index (PD) is above about 4, such as, for example, greater than about 4, in embodiments from about 4 to about 20, in embodiments from about 5 to about 10, and in embodiments from about 6 to about 8, as measured by GPC versus standard polystyrene reference resins. The PD index is the ratio of the weight-average molecular weight ( $M_w$ ) and the number-average molecular weight ( $M_n$ ). The low molecular weight amorphous polyester resins may have an acid value of from about 8 to about 20 mg KOH/g, in embodiments from about 9 to about 16 mg KOH/g, and in embodiments from about 11 to about 15 mg KOH/g. The high molecular weight amorphous polyester resins, which are available from a number of sources, can possess various melting points of, for example, from about 30° C. to about 140° C., in embodiments from about 75° C. to about 130° C., in embodiments from about 100° C. to about 125° C., and in embodiments from about 115° C. to about 124° C.

High molecular weight amorphous resins may possess a glass transition temperature of from about 53° C. to about 58° C., in embodiments from about 54.5° C. to about 57° C.

The amorphous resin is generally present in the toner composition in various suitable amounts, such as from about 60 to about 90 weight percent, in embodiments from about 50 to about 65 weight percent, of the toner or of the solids.

In embodiments, the toner composition, including the core and/or shell, may include at least one crystalline resin. As used herein, "crystalline" refers to a polyester with a three dimensional order. "Semicrystalline resins" as used herein refers to resins with a crystalline percentage of, for example, from about 10 to about 90%, in embodiments from about 12 to about 70%. Further, as used hereinafter "crystalline polyester resins" and "crystalline resins" encompass both crystalline resins and semicrystalline resins, unless otherwise specified.

In embodiments, the crystalline polyester resin is a saturated crystalline polyester resin or an unsaturated crystalline polyester resin.

For forming a crystalline polyester, suitable organic diols include aliphatic diols having from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonenediol, 1,10-decanediol, 1,12-dodecanediol, ethylene glycol, combinations thereof, and the like. The aliphatic diol may be, for example, selected in an amount of from about 40 to about 60 mole percent, in embodiments from about 42 to about 55 mole percent, in embodiments from about 45 to about 53 mole percent of the resin.

Examples of organic diacids or diesters selected for the preparation of the crystalline resins include oxalic acid, succinic acid, glutaric acid, adipic acid, suberic acid, azelaic acid, fumaric acid, maleic acid, dodecanedioic acid, sebacic acid, phthalic acid, isophthalic acid, terephthalic acid, naph-

thalene-2,6-dicarboxylic acid, naphthalene-2,7-dicarboxylic acid, cyclohexane dicarboxylic acid, malonic acid and mesaconic acid, a diester or anhydride thereof, and combinations thereof. The organic diacid may be selected in an amount of, for example, in embodiments from about 40 to about 60 mole percent, in embodiments from about 42 to about 55 mole percent, in embodiments from about 45 to about 53 mole percent.

Examples of crystalline resins include polyesters, polyamides, polyimides, polyolefins, polyethylene, polybutylene, polyisobutyrate, ethylene-propylene copolymers, ethylene-vinyl acetate copolymers, polypropylene, mixtures thereof, and the like. Specific crystalline resins may be polyester based, such as poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copoly(ethylene-adipate), poly(decylene-sebacate), poly(decylene-decanoate), poly(ethylene-decanoate), poly(ethylene-dodecanoate), poly(nonylene-sebacate), poly(nonylene-decanoate), copoly(ethylene-fumarate)-copoly(ethylene-sebacate), copoly(ethylene-fumarate)-copoly(ethylene-decanoate), copoly(ethylene-fumarate)-copoly(ethylene-dodecanoate), and combinations thereof. The crystalline resin may be present, for example, in a combined amount, including both the core and shell of the toner particles, of from about 5 to about 25 percent by weight of the toner components, in embodiments from about 6 to about 15 percent by weight of the toner components.

The crystalline polyester resins, which are available from a number of sources, may possess various melting points of, for example, from about 30° C. to about 120° C., in embodiments from about 50° C. to about 90° C. The crystalline resins may have, for example, a number average molecular weight ( $M_n$ ), as measured by gel permeation chromatography (GPC) of, for example, from about 1,000 to about 50,000, in embodiments from about 2,000 to about 25,000, in embodiments from about 3,000 to about 15,000, and in embodiments from about 6,000 to about 12,000. The weight average molecular weight ( $M_w$ ) of the resin is 50,000 or less, for example, from about 2,000 to about 50,000, in embodiments from about 3,000 to about 40,000, in embodiments from about 10,000 to about 30,000 and in embodiments from about 21,000 to about 24,000, as determined by GPC using polystyrene standards. The molecular weight distribution ( $M_w/M_n$ ) of the crystalline resin is, for example, from about 2 to about 6, in embodiments from about 3 to about 4. The crystalline polyester resins may have an acid value of about 2 to about 20 mg KOH/g, in embodiments from about 5 to about 15 mg KOH/g, and in embodiments from about 8 to about 13 mg KOH/g. The acid value (or neutralization number) is the mass of potassium hydroxide (KOH) in milligrams that is required to neutralize one gram of the crystalline polyester resin.

Suitable crystalline polyester resins include those disclosed in U.S. Pat. No. 7,329,476 and U.S. Patent Application Pub. Nos. 2006/0216626, 2008/0107990, 2008/0236446 and 2009/0047593, each of which is hereby incorporated by reference in their entirety. In embodiments, a suitable crystalline resin may include a resin composed of ethylene glycol or nonanediol and a mixture of dodecanedioic acid and fumaric acid co-monomers with the following formula (II):



wherein b is from about 5 to about 2000 and d is from about 5 to about 2000.

If semicrystalline polyester resins are employed herein, the semicrystalline resin may include poly(3-methyl-1-butene), poly(hexamethylene carbonate), poly(ethylene-p-carboxy phenoxy-butylate), poly(ethylene-vinyl acetate), poly(docosyl acrylate), poly(dodecyl acrylate), poly(octadecyl acrylate), poly(octadecyl methacrylate), poly(behenylpolyethoxyethyl methacrylate), poly(ethylene adipate), poly(decamethylene adipate), poly(decamethylene azelaate), poly(hexamethylene oxalate), poly(decamethylene oxalate), poly(ethylene oxide), poly(propylene oxide), poly(butadiene oxide), poly(decamethylene oxide), poly(decamethylene sulfide), poly(decamethylene disulfide), poly(ethylene sebacate), poly(decamethylene sebacate), poly(ethylene suberate), poly(decamethylene succinate), poly(eicosamethylene malonate), poly(ethylene-p-carboxy phenoxy-undecanoate), poly(ethylene dithionophthalate), poly(methyl ethylene terephthalate), poly(ethylene-p-carboxy phenoxy-valerate), poly(hexamethylene-4,4'-oxydibenzoate), poly(10-hydroxy capric acid), poly(isophthalaldehyde), poly(octamethylene dodecanedioate), poly(dimethyl siloxane), poly(dipropyl siloxane), poly(tetramethylene phenylene diacetate), poly(tetramethylene trithiodicarboxylate), poly(trimethylene dodecane dioate), poly(m-xylene), poly(p-xylene pimelamide), and combinations thereof.

As noted above, in embodiments a toner of the present disclosure may also include at least one high molecular weight branched or cross-linked amorphous polyester resin. This high molecular weight resin may include, in embodiments, for example, a branched amorphous resin or amorphous polyester, a cross-linked amorphous resin or amorphous polyester, or mixtures thereof, or a non-cross-linked amorphous polyester resin that has been subjected to cross-linking. In accordance with the present disclosure, from about 1% by weight to about 100% by weight of the high molecular weight amorphous polyester resin may be branched or cross-linked, in embodiments from about 2% by weight to about 50% by weight of the higher molecular weight amorphous polyester resin may be branched or cross-linked.

In accordance with the present disclosure, it has been surprisingly found that by transferring a small percentage of crystalline polyester from the core of the toner to the shell of the toner, gloss may be reduced while retaining the low melt properties of the toner. In embodiments, such improvements may be realized by forming toner particles having a core including an amorphous resin in an amount of from about 45% by weight to about 75% by weight of the core, in embodiments from about 50% by weight to about 60% by weight of the core, in embodiments about 57.5% by weight of the core. In embodiments, toner particles may have a core including a low molecular weight, high Tg, amorphous resin in an amount from about 10% by weight to about 50% by weight of the core, in embodiments from about 25% by weight to about 35% by weight of the core, in embodiments about 32.2% by weight of the core, in combination with a high molecular weight, low Tg, amorphous resin present in an amount of from about 15% by weight to about 40% by weight

of the core, in embodiments from about 25% by weight to about 35% by weight of the core, in embodiments about 25.3% by weight of the core.

The core may also include a crystalline resin in an amount of from about 4% by weight to about 15% by weight of the core, in embodiments from about 5% by weight to about 7% by weight of the core.

Such toner particles may also include a shell including an amorphous resin in an amount from about 50% by weight to about 90% by weight of the shell, in embodiments from about 60% by weight to about 80% by weight of the shell. In embodiments, the shell of the toner particles may include a combination of low molecular weight, high Tg, amorphous resins in combination with a high molecular weight, low Tg, amorphous resin.

In embodiments, the shell may also include a crystalline resin present in amounts from about 10% by weight to about 50% by weight of the shell, in embodiments from about 20% by weight to about 40% by weight of the shell.

As noted above, in embodiments, the resin may be formed by emulsion aggregation methods. Utilizing such methods, the resin may be present in a resin emulsion, which may then be combined with other components and additives to form a toner of the present disclosure.

#### Toner

The resins described above, in embodiments a combination of polyester resins, for example a low molecular weight resin, a high molecular weight resin, and a crystalline resin, may be utilized to form toner compositions. Such toner compositions may include optional colorants, waxes, and other additives. Toners may be formed utilizing any method within the purview of those skilled in the art including, but not limited to, emulsion aggregation methods.

#### Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy)ethanol, available from Rhone-Poulenc as IGEPAL CA210<sup>TM</sup>, IGEPAL CA520<sup>TM</sup>, IGEPAL CA720<sup>TM</sup>, IGEPAL CO-890<sup>TM</sup>, IGEPAL CO-720<sup>TM</sup>, IGEPAL CO-290<sup>TM</sup>, IGEPAL CA-210<sup>TM</sup>, ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, acids such as abitic acid available from Aldrich, NEOGEN R<sup>TM</sup>, NEOGEN S<sup>TM</sup> obtained from Daiichi Kogyo Seiyaku, combinations thereof, and the like. Other suitable anionic surfactants include, in embodiments, DOWFAX<sup>TM</sup> 2A1, an alkylidiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL<sup>TM</sup> and ALKAQUAT<sup>TM</sup>, available from Alkaril Chemical Company, SANIZOL<sup>TM</sup> (benzalkonium chloride), available from Kao Chemicals, and the like, and mixtures thereof.

#### Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 0.1 to about 35 percent by weight of the toner, or from about 1 to about 15 weight percent of the toner, or from about 3 to about 10 percent by weight of the toner.

As examples of suitable colorants, mention may be made of carbon black like REGAL 330<sup>®</sup>; magnetites, such as Mobay magnetites M08029<sup>TM</sup>, MO8060<sup>TM</sup>; Columbian magnetites; MAPICO BLACKS<sup>TM</sup> and surface treated magnetites; Pfizer magnetites CB4799<sup>TM</sup>, CB5300<sup>TM</sup>, CB5600<sup>TM</sup>, MCX6369<sup>TM</sup>; Bayer magnetites, BAYFERROX 8600<sup>TM</sup>, 8610<sup>TM</sup>; Northern Pigments magnetites, NP-604<sup>TM</sup>, NP-608<sup>TM</sup>; Magnox magnetites TMB-100<sup>TM</sup>, or TMB-104<sup>TM</sup>; and the like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals, HELIOGEN BLUE L6900<sup>TM</sup>, D6840<sup>TM</sup>, D7080<sup>TM</sup>, D7020<sup>TM</sup>, PYLAM OIL BLUE<sup>TM</sup>, PYLAM OIL YELLOW<sup>TM</sup>, PIGMENT BLUE 1<sup>TM</sup> available from Paul Uhlich & Company, Inc., PIGMENT VIOLET 1<sup>TM</sup>, PIGMENT RED 48<sup>TM</sup>, LEMON CHROME YELLOW DCC 1026<sup>TM</sup>, E.D. TOLUIDINE RED<sup>TM</sup> and BON RED C<sup>TM</sup> available from Dominion Color Corporation, Ltd., Toronto, Ontario, NOVAPERM YELLOW FGL<sup>TM</sup>, HOSTAPERM PINK E<sup>TM</sup> from Hoechst, and CINQUASIA MAGENTA<sup>TM</sup> available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI 60710, CI Dispersed Red 15, diazo dye identified in the Color Index as CI 26050, CI Solvent Red 19, and the

like. Illustrative examples of cyans include copper tetra(oc-tadecyl sulfonamido) phthalocyanine, x-copper phthalocya-nine pigment listed in the Color Index as CI 74160, CI Pig-ment Blue, Pigment Blue 15:3, and Anthrathrene Blue, identified in the Color Index as CI 69810, Special Blue X-2137, and the like. Illustrative examples of yellows are diarylide yellow 3,3-dichlorobenzidine acetoacetanilides, a monoazo pigment identified in the Color Index as CI 12700, CI Solvent Yellow 16, a nitrophenyl amine sulfonamide iden-tified in the Color Index as Foron Yellow SE/GLN, CI Dis-persed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK™, and cyan components may also be selected as colorants. Other known colorants can be selected, such as Levanyl Black A-SF (Miles, Bayer) and Sunperse Carbon Black LHD 9303 (Sun Chemicals), and colored dyes such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), Lithol Scarlet D3700(BASF), Toluidine Red (Ald-rich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scar-let L4300 (BASF), combinations of the foregoing, and the like.

#### Wax

In addition to the polymer binder resin and photoinitiator, the toners of the present disclosure also optionally contain a wax, which can be either a single type of wax or a mixture of two or more different waxes. A single wax can be added to toner formulations, for example, to improve particular toner properties, such as toner particle shape, presence and amount of wax on the toner particle surface, charging and/or fusing characteristics, gloss, stripping, offset properties, and the like. Alternatively, a combination of waxes can be added to provide multiple properties to the toner composition.

In accordance with the present disclosure, it has been found that a low melt toner producing a low gloss to matte finish may be obtained by including a crystalline polyester resin in the shell and a low percentage of wax. Increasing the percent-age of wax may result in poor charging of the toner particles. Where utilized, the wax may be combined with the resin in forming toner particles. When included, the wax may be present in an amount of, for example, from about 1 weight percent to about 24 weight percent of the toner particles, in embodiments from about 3 weight percent to about 10 weight percent of the toner particles.

Waxes that may be selected include waxes having, for example, a weight average molecular weight of from about 500 to about 20,000, in embodiments from about 1,000 to about 10,000. Waxes that may be used include, for example,

polyolefins such as polyethylene, polypropylene, and poly-butene waxes such as commercially available from Allied Chemical and Petrolite Corporation, for example POLY-WAX™ polyethylene waxes from Baker Petrolite, wax emulsions available from Michaelman, Inc. and the Daniels Products Company, EPOLENE N-15™ commercially available from Eastman Chemical Products, Inc., and VISCOL 550-P™, a low weight average molecular weight polypropylene available from Sanyo Kasei K. K.; plant-based waxes, such as 10 carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax, and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride dis-tearate, and pentaerythritol tetra behenate; ester waxes 20 obtained from higher fatty acid and multivalent alcohol multimers, such as diethyleneglycol monostearate, dipropylene-glycol distearate, diglyceryl distearate, and triglyceryl tetra-stearate; sorbitan higher fatty acid ester waxes, such as sorbitan monostearate, and cholesterol higher fatty acid ester waxes, such as cholestryl stearate. Examples of functionalized waxes that may be used include, for example, amines, amides, for example AQUA SUPERSLIP 6550™, SUPER-SLIP 6530™ available from Micro Powder Inc., fluorinated waxes, for example POLYFLUO 190™, POLYFLUO 200™, 30 POLYSILK 19™, POLYSILK 14™ available from Micro Powder Inc., mixed fluorinated, amide waxes, for example MICROSERSION 19™ also available from Micro Powder Inc., imides, esters, quaternary amines, carboxylic acids or acrylic polymer emulsion, for example JONCRYL 74™, 89™, 130™, 537™, and 538™, all available from SC Johnson Wax, and chlorinated polypropylenes and polyethylenes available from Allied Chemical and Petrolite Corporation and SC Johnson wax. Mixtures and combinations of the foregoing waxes may also be used in embodiments. 40 Waxes may be included as, for example, fuser roll release agents.

#### Toner Preparation

The toner particles may be prepared by any method within the purview of one skilled in the art. Although embodiments relating to toner particle production are described below with respect to emulsion aggregation processes, any suitable method of preparing toner particles may be used, including chemical processes, such as suspension and encapsulation processes disclosed in U.S. Pat. Nos. 5,290,654 and 5,302, 45 50 55 486, the disclosures of each of which are hereby incorporated by reference in their entirety. In embodiments, toner compositions and toner particles may be prepared by aggregation and coalescence processes in which small-size resin particles are aggregated to the appropriate toner particle size and then coalesced to achieve the final toner-particle shape and morphology.

In embodiments, toner compositions may be prepared by emulsion aggregation processes, such as a process that includes aggregating a mixture of an optional wax and any other desired or required additives, and emulsions including the resins described above, optionally in surfactants as described above, and then coalescing the aggregate mixture. A mixture may be prepared by adding an optional wax or other materials, which may also be optionally in a dispersion (s) including a surfactant, to the emulsion, which may be a mixture of two or more emulsions containing the resin(s). The pH of the resulting mixture may be adjusted by an acid such

as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1 parts per hundred (pph) to about 1 pph, in embodiments from about 0.25 pph to about 0.75 pph, in some embodiments about 0.5 pph. This provides a sufficient amount of agent for aggregation.

The gloss of a toner may be influenced by the amount of retained metal ion, such as Al<sup>3+</sup>, in the particle. The amount of retained metal ion may be further adjusted by the addition of EDTA. In embodiments, the amount of retained crosslinker, for example Al<sup>3+</sup>, in toner particles of the present disclosure may be from about 0.1 pph to about 3 pph, in embodiments from about 0.25 pph to about 2 pph, in embodiments about 1.5 pph.

In order to control aggregation and coalescence of the particles, in embodiments the aggregating agent may be metered into the mixture over time. For example, the agent may be metered into the mixture over a period of from about 5 to about 240 minutes, in embodiments from about 30 to about 200 minutes. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 40° C. to about 100° C., and holding the mixture at this temperature for a time from about 0.5 hours to about 6 hours, in embodiments from about hour 1 to about 5 hours, while maintaining stirring, to provide the

aggregated particles. Once the predetermined desired particle size is reached, then the growth process is halted. In embodiments, the predetermined desired particle size is within the toner particle size ranges mentioned above.

5 The growth and shaping of the particles following addition of the aggregation agent may be accomplished under any suitable conditions. For example, the growth and shaping may be conducted under conditions in which aggregation occurs separate from coalescence. For separate aggregation 10 and coalescence stages, the aggregation process may be conducted under thermal conditions at an elevated temperature, for example of from about 40° C. to about 90° C., in embodiments from about 45° C. to about 63° C., which may be below the glass transition temperature of the resin as discussed 15 above.

In embodiments, the aggregate particles may have a volume average diameter (also referred to as "volume average particle diameter") of less than about 5 microns, in embodiments from about 4 microns to about 5 microns, in embodiments 20 from about 4.5 microns to about 4.9 microns.

#### Shell Resin

In embodiments, a shell may be applied to the formed aggregated toner particles. Any resin described above as suitable for the core resin may be utilized as the shell resin. The 25 shell resin may be applied to the aggregated particles by any method within the purview of those skilled in the art. In embodiments, the shell resin may be in an emulsion including any surfactant described above. The aggregated particles described above may be combined with said emulsion so that 30 the resin forms a shell over the formed aggregates. In embodiments, an amorphous polyester and a crystalline resin may be utilized to form a shell over the aggregates to form toner particles having a core-shell configuration.

The shell resin may be present in an amount of from about 35 5 percent to about 40 percent by weight of the toner particles, in embodiments from about 24 percent to about 30 percent by weight of the toner particles.

Once the desired final size of the toner particles is achieved, the pH of the mixture may be adjusted with a base to a value 40 of from about 5 to about 10, and in embodiments from about 6 to about 8. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above. The base may be added in amounts from about 2 to about 25 percent by weight of the mixture, in embodiments from about 4 to about 10 percent by weight of the mixture.

#### Coalescence

Following aggregation to the desired particle size, with the formation of an optional shell as described above, the particles 55 may then be coalesced to the desired final shape, the coalescence being achieved by, for example, heating the mixture to a temperature of from about 55° C. to about 100° C., in embodiments from about 65° C. to about 90° C., in embodiments about 85° C., which may be below the melting point of the crystalline resin to prevent plasticization. Higher or lower temperatures may be used, it being understood that the temperature is a function of the resins used for the binder.

Coalescence may proceed and be accomplished over a period of from about 0.1 to about 9 hours, in embodiments 60 from about 0.5 to about 4 hours.

After coalescence, the mixture may be cooled to a lower temperature, such as from about 20° C. to about 40° C. The

cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

#### Additives

In embodiments, the toner particles may also contain other optional additives, as desired or required. For example, the toner may include any known charge additives in amounts of from about 0.1 to about 10 weight percent, and in embodiments of from about 0.5 to about 7 weight percent of the toner. Examples of such charge additives include alkyl pyridinium halides, bisulfates, the charge control additives of U.S. Pat. Nos. 3,944,493, 4,007,293, 4,079,014, 4,394,430 and 4,560,635, the disclosures of each of which are hereby incorporated by reference in their entirety, negative charge enhancing additives like aluminum complexes, and the like.

Surface additives can be added to the toner compositions of the present disclosure after washing or drying. Examples of such surface additives include, for example, metal salts, metal salts of fatty acids, colloidal silicas, metal oxides, strontium titanates, mixtures thereof, and the like. Surface additives may be present in an amount of from about 0.1 to about 10 weight percent, and in embodiments of from about 0.5 to about 7 weight percent of the toner. Examples of such additives include those disclosed in U.S. Pat. Nos. 3,590,000, 3,720,617, 3,655,374 and 3,983,045, the disclosures of each of which are hereby incorporated by reference in their entirety. Other additives include zinc stearate and AEROSIL R972® available from Degussa. The coated silicas of U.S. Pat. Nos. 6,190,815 and 6,004,714, the disclosures of each of which are hereby incorporated by reference in their entirety, can also be present in an amount of from about 0.05 to about 5 percent, and in embodiments of from about 0.1 to about 2 percent of the toner, which additives can be added during the aggregation or blended into the formed toner product.

The characteristics of the toner particles may be determined by any suitable technique and apparatus. Volume average particle diameter  $D_{50v}$ , GSDv, and GSDn may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3. Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH. Toners of the present disclosure may also possess a parent toner charge per mass ratio (Q/M) of from about  $-3 \mu\text{C/g}$  to about  $-35 \mu\text{C/g}$ , and a final toner charging after surface additive blending of from  $-10 \mu\text{C/g}$  to about  $-45 \mu\text{C/g}$ .

Utilizing the methods of the present disclosure, the toner formulation design may be adjusted so that the levels of glossiness become tunable. As noted above, this may be accomplished by relocating a certain amount of crystalline resin in the toner during the aggregation and coalescence process from the core to the shell. Thus, for example, the gloss level of a toner of the present disclosure may have a gloss as measured in Gardner Gloss Units (ggu) by a Gardner 75° Gloss Meter, of from about 25 ggu to about 85 ggu, in embodiments from about 35 ggu to about 75 ggu.

In embodiments, toners of the present disclosure may be utilized as ultra low melt (ULM) toners. In embodiments, the dry toner particles, exclusive of external surface additives, may have the following characteristics:

5 (1) Volume average diameter of from about 2.5 to about 20 microns, in embodiments from about 2.75 to about 18 microns, in other embodiments from about 3 to about 15 microns.

10 (2) Number Average Geometric Standard Deviation (GSDn) and/or Volume Average Geometric Standard Deviation (GSDv) of from about 1.18 to about 1.35, in embodiments from about 1.20 to about 1.34.

15 (3) Circularity of from about 0.9 to about 1 (measured with, for example, a Sysmex FPIA 2100 analyzer), in embodiments from about 0.95 to about 0.985, in other embodiments from about 0.96 to about 0.98.

20 (4) A minimum fixing temperature of from about 120° C. to about 160° C., in embodiments from about 130° C. to about 150° C.

#### Developers

The toner particles thus formed may be formulated into a developer composition. The toner particles may be mixed with carrier particles to achieve a two-component developer composition. The toner concentration in the developer may be 25 from about 1% to about 25% by weight of the total weight of the developer, in embodiments from about 2% to about 15% by weight of the total weight of the developer.

#### Carriers

30 Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and 35 the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a 40 mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and 45 the like. For example, coatings containing polyvinylidene-fluoride, available, for example, as KYNAR 301F™, and/or polymethylmethacrylate, for example having a weight average molecular weight of about 300,000 to about 350,000, such as commercially available from Soken, may be used. In 50 embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a 55 coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting 60 copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may 65 be prepared by mixing the carrier core with polymer in an amount from about 0.05 to about 10 percent by weight, in embodiments from about 0.01 percent to about 3 percent by

weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu\text{m}$  in size, in embodiments from about 50 to about 75  $\mu\text{m}$  in size, coated with about 0.5% to about 10% by weight, in embodiments from about 0.7% to about 5% by weight of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

## Imaging

The toners can be utilized for electrophotographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengerless development (HSD), and the like. These and similar development systems are within the purview of those skilled in the art.

Imaging processes include, for example, preparing an image with an electrophotographic device including a charging component, an imaging component, a photoconductive component, a developing component, a transfer component, and a fusing component. In embodiments, the development component may include a developer prepared by mixing a carrier with a toner composition described herein. The electrophotographic device may include a high speed printer, a black and white high speed printer, a color printer, and the like.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser member. The fusing member can be of any desired or suitable configuration, such as a drum or roller, a belt or web, a flat surface or platen, or the like. The fusing member can be applied to the image by any desired or suitable method, such as by passing the final recording substrate through a nip formed by the fusing member and a back member, which can be of any desired or effective configuration, such as a drum or roller, a belt or web, a flat surface or platen, or the like. In embodiments, a fuser roll can be used. Fuser roll members are contact fusing devices that are within the purview of those skilled in the art, in which pressure from the roll, optionally with the application of heat, may be used to fuse the toner to the

image-receiving medium. Optionally, a layer of a liquid such as a fuser oil can be applied to the fuser member prior to fusing.

In embodiments, the toner image can be fused by cold pressure fusing, i.e., without the application of heat. Fusing can be effected at any desired or effective pressure, in embodiments from about 1000 pounds per square inch (psi) to about 10,000 pounds per square inch, in embodiments from about 1,500 pounds per square inch to about 5,000 pounds per square inch. One advantage with cold pressure fusing is that it requires low power, and unlike hot roll processes, no standby power. Thus, toners of the present disclosure may be utilized in systems that are more environmentally friendly, having lower energy requirements. Moreover, as heat is not applied to the toners, the toners do not become molten and thus do not offset during fusing.

Toners of the present disclosure may have excellent blocking, i.e., the ability of the toner to resist sticking together during shipping and/or storage.

20 The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 30° C.

## EXAMPLES

### Comparative Example 1

A cyan polyester emulsion aggregation toner was prepared without a crystalline resin in the shell. A cyan polyester toner was prepared at a 2 liter bench scale (about 150 grams dry theoretical toner). The core toner slurry included two amorphous polyester resin emulsions (at a ratio of about 50:50). One emulsion included a low molecular weight resin including an alkoxylated Bisphenol A with terephthalic acid, fumaric acid, and dodecenyldsuccinic acid co-monomers, and the other emulsion included a high molecular weight resin including alkoxylated Bisphenol A with terephthalic acid, trimellitic acid, and dodecenyldsuccinic acid co-monomers. Added thereto was about 6.8% weight percent of a crystalline resin of the following formula:



wherein b was from about 5 to about 2000 and d was from about 5 to about 2000, DOWFAX™ 2A1, an alkylidiphenyloxide disulfonate available commercially from The Dow Chemical Company, about 5.5% of a cyan pigment (Pigment Blue 15:3) in a dispersion, and about 9% of a polyethylene wax (from IGI) in a dispersion. The components were mixed and then pH adjusted to 4.2 using 0.3M nitric acid.

60 The slurry was then homogenized for about 10 minutes at from about 3000 revolutions per minute (rpm) to about 6000 rpm while adding about 0.5 ppm of aluminum sulfate as a coagulant. The toner slurry was then transferred to the 2 liter Buchi reactor and heated to begin aggregation. The toner slurry aggregated at a temperature of around 43° C. During aggregation, the toner particle size was closely monitored. At around 4.8 microns in size, a shell including the same amor-

65

19

phous emulsion (ratio 50:50) as in the core was added to achieve the final targeted particle size of about 5.8 microns. The pH of the slurry was adjusted to about 7.5 using sodium hydroxide (NaOH) and VERSENE-100 from the Dow Chemical Company to freeze, i.e. stop, the aggregation step.

The process proceeded with the reactor temperature (Tr) increased to achieve 85° C. while maintaining a pH $\geq$ about 7.5 until Tr was about 85° C. Once the Tr reached 85° C., the pH of the toner slurry was reduced to 7 with the addition of diluted nitric acid and held until the circularity reached  $\geq$ about 0.960.

The final toner particle had a particle size (D50), particle distribution by volume, and circularity of 6.15 microns, 1.26 and 0.970, respectively. Toner particles were tested as described below, with the results set forth in the Figures.

### Example 1

A cyan polyester emulsion aggregation toner was prepared with a crystalline resin in the shell. A cyan polyester toner was prepared at a 2 liter bench scale (about 150 grams dry theoretical toner). About 25.3% by weight of a high molecular weight amorphous resin and about 32.2% by weight of a low molecular weight amorphous resin as described above in Comparative Example 1 were combined with DOWFAX™ 2A1, an alkylidiphenyloxide disulfonate available commercially from The Dow Chemical Company, about 5.5% by weight of a cyan pigment (Pigment Blue 15:3) in a dispersion, and about 9% of a polyethylene wax (from IGI) in a dispersion. The components were mixed and then pH adjusted to about 4.2 using about 0.3M nitric acid.

The slurry was then homogenized for about 10 minutes at from about 3000 revolutions per minute (rpm) to about 6000 rpm while adding about 0.5 ppm of aluminum sulfate as a coagulant. The toner slurry was then transferred to the 2 liter Buchi reactor and heated to begin aggregation. The toner slurry aggregated at a temperature of around 43° C. During aggregation, the toner particle size was closely monitored. At around 4.8 microns in size, a shell including the 14% by weight of the high molecular weight amorphous resin, 7.2% by weight of the low molecular weight amorphous resin in emulsion, and about 6.8% by weight of crystalline resin was added in an emulsion to achieve the final targeted particle size of about 5.8 microns. The pH of the slurry was adjusted to about 7.5 using sodium hydroxide (NaOH) and VERSENE-100 from the Dow Chemical Company to freeze, i.e. stop, the aggregation step.

As in Comparative Example 1, the process proceeded with the reactor temperature (Tr) increased to achieve 85° C. while maintaining a pH $\geq$ about 7.5 until Tr was about 85° C. Once the Tr reached 85° C., the pH of the toner slurry was reduced to 7 with the addition of diluted nitric acid and held until the circularity reached  $\geq$ about 0.960.

The final toner particle had a particle size (D50), particle distribution by volume, and circularity of 8.33 microns, 1.31 and 0.967, respectively.

### Example 2

The process of Example 1 was repeated to form a cyan polyester toner with a crystalline resin in the shell. About 6.8% by weight of the same crystalline resin was used as in Example 1, formed by a solvent-free process as disclosed in U.S. Patent Application Publication Nos. 20080138738 and 20080138739, the disclosures of each of which are hereby incorporated by reference in their entirety, while the crystalline resin of Example 2 was produced by a phase inversion

20

emulsification process as disclosed in U.S. patent application Ser. No. 12/778,431 filed May 12, 2010, the disclosure of which is hereby incorporated by reference in its entirety.

The only other difference between this Example 2 and Example 1 is that the coalescence occurred at 75° C., instead of 85° C. as in Example 1.

### Fusing

The toners of Comparative Example 1, Example 1, and Example 2 were submitted for fusing evaluation. Fusing performance (gloss, crease, and hot offset measurements) of particles was collected.

All unfused images were generated using a modified DC12 copier from Xerox Corporation. A TMA (Toner Mass per unit Area) of 1.00 mg/cm<sup>2</sup> of each toner was made on Color Xpressions+ paper (90 gsm, uncoated) (sometimes referred to as CX+ paper), using a commercially available fusing fixture. Gloss/crease targets were a square image placed in the center of the page.

Process speed of the fuser was set to 220 mm/second (nip dwell of about 34 milliseconds) and the fuser roll temperature was varied from cold offset to hot offset or up to about 210° C. for gloss and crease measurements.

Crease area measurements were carried out with an image analysis system. Print gloss as a function of fuser roll temperature was measured with a BYK Gardner 75° gloss meter. A summary of the fusing results is reported in Table 1 below. Gloss at 185° C., fusing latitude, and the minimum fusing temperature (MFT) are reported.

TABLE 1

| On CX+                              | Fusing Summary        |                |                |
|-------------------------------------|-----------------------|----------------|----------------|
|                                     | Comparative Example 1 | Example 1      | Example 2      |
| A1 content (ppm)                    | 60                    | 139            | 122            |
| Cold offset                         | 120                   | 123            | 120            |
| Gloss at MFT                        | 27.4                  | 10.8           | 20.3           |
| Gloss at 185°                       | 73.5                  | 44.1           | 40.8           |
| Peak Gloss                          | 74.4                  | 48.4           | 58.9           |
| MFT <sub>C4-80</sub> (extrapolated) | 123                   | 126            | 119            |
| ΔMFT                                | -27                   | -25            | -35            |
| Fusing Latitude HO-MFT on CX+ (>50) | 72                    | 84             | 91             |
| D50 (microns)/GSDV/GSDn             | 5.89/1.22/1.23        | 8.33/1.31/1.33 | 7.05/1.30/1.44 |

As can be seen from Table 1, when the toner of Example 1 was compared to the toner of Comparative Example 1, the gloss at MFT, 185° C., and Peak Gloss were all lower in Example 1 than in the Comparative Example 1. The toner of Example 1 also exhibited higher fusing latitude.

As shown in FIG. 1, the addition of a crystalline emulsion to the shell of the toner produced a lower gloss toner while maintaining the ultra low melt properties of the toner.

As shown in FIG. 2, the low melt performance was maintained with CPE in the shell. (The crease area depicted in FIG. 2 is a measurement of adhesion to the substrate with low fuser roll temperatures, with low crease area desired.) As shown in FIG. 2, the two examples with CPE in the shell were within experimental uncertainty of the comparative toner made with CPE in the core.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in

21

the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A toner comprising particles comprising:  
a core comprising at least one amorphous polyester resin,  
an optional crystalline resin, a colorant, and an optional  
wax; and  
a shell comprising, at least one amorphous resin in combi-  
nation with at least one crystalline resin, the at least one  
crystalline resin being present in an amount of from 1%  
to 50% by weight of the shell,  
wherein the toner has a gloss of from 25 ggu to 85 ggu.
  2. The toner according to claim 1, wherein the at least one  
amorphous polyester resin comprises an alkoxylated bisphe-  
ol A fumarate/terephthalate based polyester or copolyester  
resin.
  3. The toner according to claim 1, wherein the crystalline  
resin is of the formula:



wherein b is from 5 to about 2000 and d is from about 5 to about 2000.

4. The toner according to claim 1, wherein the core comprises a second amorphous resin.
  5. The toner according to claim 1, wherein the shell comprises from 50% to 90% by weight of at least one amorphous resin.
  6. The toner according to claim 1, wherein the core further comprises a wax, the wax being present in an amount of from 1% to 24% by weight of the toner.
  7. The toner according to claim 6, wherein the core

7. The toner according to claim 6, wherein the wax is selected from the group consisting of polyethylene wax, polypropylene wax, polybutene wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentaerythritol tetra behenate, diethyleneglycol monostearate, dipropyleneglycol distearate, and combinations thereof, and wherein the wax is present in an amount of from 3 percent to 10 percent by weight of the toner.

8. The toner according to claim 1, wherein the crystalline resin is present in an amount from 10% to 50% by weight of the shell.

9. The toner according to claim 1, wherein the toner has a gloss of from 35 ggu to 75 ggu, and a minimum fixing temperature of from 120° C. to 160° C.

10. A toner comprising particles comprising:  
a core comprising at least one amorphous polyester resin,  
an optional crystalline polyester resin, at least one wax,  
and a colorant; and

22

a shell comprising at least one amorphous resin in combination with at least one crystalline resin, the at least one crystalline resin being present in an amount of from 1% to 50% by weight of the shell,

- 5 wherein the toner has a gloss of from 35 ggu to 75 ggu.

11. The toner according to claim 10, wherein the at least one amorphous polyester resin comprises an alkoxylated bisphenol A fumarate/terephthalate based polyester or copolyester resin.

10 12. The toner according to claim 10, wherein the crystalline polyester resin is of the formula:



wherein  $b$  is from 5 to 2000 and  $d$  is from 5 to 2000

13. The toner according to claim 10, wherein the at least one amorphous polyester resin is present in an amount from 50% to 90% by weight of the shell, and wherein the crystalline polyester resin is present in the shell in an amount of from 10% to 50% by weight of the shell.

14. The toner according to claim 10, wherein the wax is present in an amount of from 3 percent to 10 percent by weight of the toner.

15. The toner according to claim 10, wherein the toner has a minimum fixing temperature of from 120° C. to 160° C.
  16. A toner comprising:

a core comprising at least one amorphous polyester resin, from 1% to 24% by weight of at least one wax, and at least one colorant; and a shell comprising from 50% to 90% by weight of at least one amorphous polyester resin, and from 10% to 50% of at least one crystalline resin, wherein the taper has a slope from 25 cm to about 85 cm.

17. The toner according to claim 16, wherein the shell comprises from 60% to 80% by weight of the at least one amorphous resin and from 20% to 40% of the crystalline resin.

18. The toner according to claim 16, wherein the wax is present in an amount of from 3 percent to 10 percent by weight of the toner.

- 19.** The toner according to claim **16**, wherein the crystalline resin comprises a crystalline resin of the formula:



wherein b is from 5 to 2000 and d is from 5 to 2000.

- 20.** The toner according to claim 16, wherein the toner has a minimum fixing temperature of from 120° C. to 160° C.

\* \* \* \*